

1

2,750,282

STAINLESS STEEL OF THE "20" TYPE

Norman S. Mott, Westfield, N. J., assignor to Cooper Alloy Corporation, Hillside, N. J., a corporation of New Jersey

No Drawing. Application April 11, 1955,  
Serial No. 500,693

14 Claims. (Cl. 75—125)

This invention relates to stainless steel, and more particularly to stainless steel of the "20" type.

A most popular stainless steel alloy with greater corrosion resistance than either the "304" or "316" types of the American Iron and Steel Institute (AISI) is a high chromium-nickel-copper-molybdenum alloy generally known as the "20" alloy. This has the approximate analysis 20% chromium, 28% nickel, 3.5% copper and 3% molybdenum.

This alloy is in great demand and is extensively used in the chemical and associated industries where corrosive conditions are more exacting, and where sufficient corrosion resistance cannot be had by using such chromium-nickel and chromium-nickel-molybdenum types as AISI "304" and "316." Unfortunately this "20" alloy has a relatively low hardness, even lower than the "304" and "316" types, and this low hardness has produced extreme cases of galling. This precludes its successful use in corrosion resisting valves, because successive opening and closing has resulted in severe tearing and scoring of the mating seat and disc surfaces. Such galling has resulted also in other applications such as bearings where surfaces are required to slide under load.

In industry it is an accepted fact that any tendency toward galling in stainless steel may be reduced to a point where mating surfaces will successfully operate without galling if there is a difference of 50 BHN or more in hardness between the mating surfaces. Such an increase of 50 BHN in hardness is considered just passing, and a greater hardness increase, such as 75 to 100 BHN more surely guarantees successful operation without galling.

The primary object of this invention is to overcome the difficulty of galling and seizing in the "20" type alloy by increasing the hardness of one of the mating parts by 50 or more points of Brinell hardness.

My new alloy of the basic "20" type analysis may be made hard enough to obviate galling difficulty through the introduction of suitable amounts of nitrogen and columbium to the composition, and then heat treating to develop their full hardening effect. In this condition the alloy fully meets the usual high standards of corrosion resistance for a "20" type alloy, and may be used in contact with the original or base "20" metal alloy without galling.

My new alloy is an alloy of the "20" type which has been hardened by the addition of .06 to .25% nitrogen, and also columbium in an amount eight or more times the carbon content, but not to exceed 1%, specifically, in a range of .20 to 1% (or .20 to 1.35% of columbium plus tantalum combined), and by further heat treating

2

the alloy in a so-called stabilizing temperature range, namely 1550° to 1650° F. for two to four or more hours, preferably about four hours, until maximum hardness is produced.

5 The heat hardening step follows a water quenching operation which preferably consists of heating the work at a temperature of from 1950° to 2050° F. (preferably 2000° F.) for a period of about one hour per inch thickness, after reaching temperature, and then water quenching.

Before giving examples of my improved alloy, it may be well to preliminarily show the effect of the addition of either nitrogen alone or columbium alone. For this purpose reference may be made to the following table:

Table I

| Test #             | Ex. #1 | Ex. #2 | Ex. #3 |
|--------------------|--------|--------|--------|
| Chemical Analysis: |        |        |        |
| C                  | .058   | .044   | .053   |
| Cr                 | 19.98  | 20.15  | 19.93  |
| Ni                 | 28.30  | 28.45  | 18.60  |
| Si                 | 1.73   | 1.98   | 1.65   |
| Mn                 | .95    | .67    | .68    |
| Cu                 | 3.04   | 3.06   | 3.04   |
| Mo                 | 3.57   | 3.78   | 3.80   |
| Ob                 |        | .77    |        |
| N <sub>2</sub>     | .052   | .126   | .013   |
| BHN:               |        |        |        |
| WQ                 | 131    | 170    | 131    |
| H                  | 152    | 229    | 170    |
| Increase over 131  | +21    | +98    | +39    |

15 In the foregoing and succeeding table "BHN" means Brinell hardness number; "WQ" means water quenched after heating for one hour at 2000° F.; and "H" means hardened by heating at 1550° F. for four hours, followed by air cooling.

20 Example #1 shows the presence of about the maximum nitrogen content found in a commercial arc-melted heat. Columbium is not present in this alloy. The BHN number of 131 may be considered to be the basic water quench hardness. The heat treatment in the stabilizing temperature range has increased the Brinell hardness by 21 points. However, this alloy is not satisfactory for heat hardening because the alloy will corrode severely after being given the hardening heat treatment.

25 Example #2 is another alloy without columbium, and in this alloy the nitrogen content has been greatly increased. It will be noted that the heat treatment has correspondingly greatly increased the BHN number to a value of 229, or an increase of 98 over the basic number of 131. This example shows that increasing the nitrogen content increases the hardness, especially after heat treatment. However, here again it is found that the alloy is subject to severe corrosion after being given the heat treatment.

30 In Example #3 a substantial quantity of columbium has been added, but nitrogen has not been added, and the nitrogen content is small. There was no increase in hardness compared to Example #1 after water quenching. There was some but not sufficient increase in hardness after the hardening heat treatment. However, this alloy was corrosion-resistant even after the hardening heat treatment.

35 The effect of increasing the nitrogen content in alloys which also have a substantial amount of columbium is illustrated in the following four examples of my invention:

**3**  
*Table II*

| Test #                 | Ex. #4 | Ex. #5 | Ex. #6 | Ex. #7 |
|------------------------|--------|--------|--------|--------|
| Chemical Analysis:     |        |        |        |        |
| C-----                 | .039   | .058   | .057   | .058   |
| Cr-----                | 20.10  | 19.93  | 20.15  | 19.75  |
| Ni-----                | 28.30  | 28.60  | 28.10  | 27.90  |
| Si-----                | 1.81   | 1.65   | 1.96   | 1.92   |
| Mn-----                | .47    | .68    | .64    | .57    |
| Cu-----                | 3.00   | 3.04   | 3.02   | 3.15   |
| Mo-----                | 3.63   | 3.80   | 3.63   | 3.95   |
| Cb-----                | .79    | .77    | .79    | .80    |
| N2-----                | .060   | .097   | .120   | .250   |
| BHN:                   |        |        |        |        |
| WQ-----                | 156    | 170    | 187    | 192    |
| H-----                 | 187    | 207    | 229    | 255    |
| Increase over 131----- | +56    | +76    | +98    | +124   |

In Example #4 the nitrogen content has been increased to 0.06 and it will be seen that the hardness after heat treatment has been raised by 56 points over the hardness number of 131 in Examples #1 and #3. This would be adequate to prevent galling.

In Example #5 the nitrogen in the columbium bearing alloy has been raised to 0.097 and the BHN has increased by 76 points over the hardness number of 131 in Examples #1 and #3.

In alloy #6 the nitrogen content has been increased to 0.129 and the BHN has increased by 98 points over the hardness number 131 in Examples #1 and #3.

In Example #7 the nitrogen content has been increased to 0.25 and the BHN has been raised by 124 points over the hardness number of 131 in Examples #1 and #3.

Alloy #7 represents the maximum amount of nitrogen that it would be feasible to add, for any higher nitrogen content results in metal which is porous because of gas holes. As a matter of fact the nitrogen content of 0.129 in Example #6 constitutes a more desirable value for nitrogen, and the hardness increase of 98 points is more than adequate to prevent galling.

In the case of a valve, the valve body member would ordinarily be made of the softer metal, specifically an alloy such as the #1 alloy, with no columbium, and solution annealed by water quenching only. With such treatment the alloy has the excellent corrosion resistance for which it is known. The valve seat disc would be made of the harder metal of my invention, including columbium and increased nitrogen, and subjected to the heat hardening treatment as well as a preceding water quenching treatment. The heat hardening may be performed in a range of, say, 1550 to 1650° F., the lower part of the range, say 1550° F., being preferred.

In the case of a shaft and bearing the shaft would ordinarily be made of the softer metal, that is a conventional #20 alloy such as Example #1 above, subjected to water quenching but not heat hardening, and the bearing would be made of my new alloy, including columbium and increased nitrogen, and subjected to heat hardening after water quenching.

It will be understood that an ordinary #20 alloy does not include columbium. However, columbium has been added in a #20 type alloy to obviate inter-granular corrosion following a welding operation. Thus, in situations in which it was anticipated that welding would have to be performed, it was known to be desirable to add columbium. However, in these alloys there was no increase in nitrogen content.

In the usual manufactured condition the "20" type alloy may have a nitrogen content of from 0.01 to 0.05%. The small nitrogen content was a natural or inevitable consequence of the normal melting procedure. However, so far as I am aware, neither columbium nor nitrogen have been added to increase hardness. A high nitrogen content has not existed in the alloy, and could result only after a deliberate and purposeful addition of a high nitrogen bearing ferro-alloy, which has not been done heretofore.

The alloy here disclosed is primarily a casting alloy. The AISI does not have a specified or standardized analysis

## 4

for the #20 alloy, but the Alloy Casting Institute (ACI) does. In this analysis the carbon is to be 0.07 maximum; the chromium is to be 18 to 22%; and the nickel 21 to 31%. Other elements, specifically silicon, molybdenum, copper and manganese, are stated to vary according to proprietary formulas. In my new alloy I recommend molybdenum to range from 2 to 4%, and copper to range from 3 to 4%, these being the ranges found in the trade alloys "FA-20," "Carpenter 20," "Durimet 20," etc.

I consider silicon and manganese to be optional, with the silicon to have a maximum limit of 2%, and the manganese to have a maximum limit of 2½%. These elements ordinarily are controlled by other factors. For example, the silicon content may be at the higher end of the 0 to 2% range when casting small castings, compared to large castings. In accordance with my invention the foregoing analysis for a #20 alloy has added thereto columbium in an amount at least eight times the carbon content, but not to exceed 1%, and nitrogen in an amount ranging from 0.06% to 0.25%.

It is believed that the composition and behavior of my improved heat hardenable high corrosion resistance stainless steel alloy, as well as the advantages thereof, will be apparent from the foregoing detailed description.

Examples #1 to #7 inclusive illustrate the effect of additions of nitrogen and columbium to an alloy having the "20" type of analysis. With that analysis the basic hardness is close to 131 BHN, after water quenching, with or without columbium. The 131 BHN hardness is obtained in the water quenched condition after heating for a period of one hour per inch, at 2000° F.

The heating may be in a temperature range from 1950 to 2050° F., with a preferred temperature of 2000° F. The period of one hour per inch means after reaching temperature, and usually is a one hour minimum even if the work being treated is less than one inch in thickness. Usually the work is non-uniform in thickness, and the timing is adjusted to the greater thickness. The water quenched condition is the condition for the best corrosion resistance when columbium is not present, as in Example #1. When columbium is present in the correct amount, as in Example #3, the alloy may be subjected to a stabilizing heat hardening treatment, such as heating for two to four hours at 1550 to 1650° F., followed by air or furnace cooling. This heat hardening may follow the water quenching operation, and the desired corrosion resistance is maintained successfully. In Example #3 the hardness is increased, but not enough to prevent galling.

In Examples #4, #5, #6 and #7 both nitrogen and columbium are present, with the nitrogen increased beyond its normal content by adding a high nitrogen ferro-chrome material to the melt. This, combined with heat hardening by a stabilizing heat treatment, raises the hardness more than enough to prevent galling. One valve or machine part is made of a standard "20" alloy, water quenched. The other rubbing part is made of my new alloy, heat hardened.

It will be apparent that while I have set forth specific examples of my improved alloy, changes may be made, without departing from the scope of the invention, as sought to be defined in the following claims.

I claim:

1. A heat hardenable high corrosion resistance alloy, said alloy consisting essentially of a chromium-nickel-copper-molybdenum stainless steel of the type known commercially as the #20 type (having an approximate analysis of 20% chromium, 28% nickel, 3.5% copper, and 3% molybdenum), said steel having added thereto columbium and nitrogen, the columbium ranging from 0.20 to 1.00%, and the nitrogen ranging from 0.06 to 0.25%.

2. A heat hardenable high corrosion resistance alloy, said alloy consisting essentially of a chromium-nickel-copper-molybdenum stainless steel of the type known commercially as the #20 type (having an approximate analysis of 20% chromium, 28% nickel, 3.5% copper,

and 3% molybdenum), said steel having added thereto columbium and nitrogen, the columbium ranging from 0.20 to 1.00%, and the nitrogen ranging from 0.06 to 0.25%, said alloy being hardenable while retaining high corrosion resistance by a hardening operation consisting of heating at about 2000° F., water quenching, and then heat hardening at about 1550° F.

3. A heat hardenable alloy of high corrosion resistance, said alloy consisting essentially of a chromium-nickel-copper-molybdenum alloy of the type known commercially as the #20 type (having an approximate analysis of 20% chromium, 28% nickel, 3.5% copper, and 3% molybdenum), said steel having columbium in an amount at least eight times the carbon content and not over 1%, and having nitrogen in a range of from 0.06% to 0.25%. 15

4. A heat hardenable alloy of high corrosion resistance, said alloy consisting essentially of a chromium-nickel-copper-molybdenum alloy of the type known commercially as the #20 type (having an approximate analysis of 20% chromium, 28% nickel, 3.5% copper, and 3% molybdenum), said steel having columbium in a range of from 0.2 to 1% and having nitrogen in a range of from 0.06% to 0.25%, and the carbon content being less than one-eighth the columbium content. 20

5. A heat hardenable alloy of high corrosion resistance, said alloy consisting essentially of a chromium-nickel-copper-molybdenum alloy of the type known commercially as the #20 type (having an approximate analysis of 20% chromium, 28% nickel, 3.5% copper, and 3% molybdenum), said steel having columbium in a range of from 0.2 to 1% and having nitrogen in a range of from 0.06% to 0.25%, the columbium content being at least eight times the carbon content, and said alloy being heat hardenable to a BHN hardness at least fifty points higher than a conventional #20 type alloy while retaining high corrosion resistance, so that the two alloys may be used in rubbing engagement without galling. 25

6. A heat hardenable high corrosion resistance stainless steel alloy of the #20 type, said alloy having about 20% chromium, 28% nickel, 3.5% copper, 3% molybdenum, 0.20 to 1.00% columbium, 0.06 to 0.25% nitrogen, the remainder being essentially iron with other ingredients common to the #20 type alloy. 40

7. A heat hardenable high corrosion resistance stainless steel alloy of the #20 type, said alloy having a range of from about 18 to 22% chromium, 21 to 31% nickel, 0 to 2% silicon, 0 to 2½% manganese, 3 to 4% copper, 2 to 4% molybdenum, 0.20 to 1.00% columbium, 0.06 to 0.25% nitrogen, the remainder being essentially iron with a carbon content not exceeding about 0.07%. 45

8. A heat hardenable high corrosion resistance stainless steel alloy of the #20 type, said alloy having a range of from about 18 to 22% chromium, 21 to 31% nickel, 0 to 2% silicon, 0 to 2½% manganese, 3 to 4% copper, 3 to 4% molybdenum, 0.06 to 0.25% nitrogen, carbon in an amount not exceeding about 0.07%, and columbium in an amount at least eight times the carbon but not exceeding 1%, the remainder being essentially iron. 50

9. A heat hardenable high corrosion resistance stainless steel alloy of the #20 type, said alloy having approximately the following chemical analysis: carbon 0.039%, chromium 20.10%, nickel 28.30%, silicon 1.81%, manganese 0.47%, copper 3.00%, molybdenum 3.63%, columbium 0.79%, nitrogen 0.06%, and the balance of the alloy being substantially all iron.

10. A heat hardenable high corrosion resistance stainless steel alloy of the #20 type, said alloy having approximately the following chemical analysis: carbon 0.053%, chromium 19.93%, nickel 28.60%, silicon 1.65%, manganese 0.68%, copper 3.04%, molybdenum 3.80%, columbium 0.77%, nitrogen 0.097%, and the balance of the alloy being substantially all iron. 10

11. A heat hardenable high corrosion resistance stainless steel alloy of the #20 type, said alloy having approximately the following chemical analysis: carbon 0.057%, chromium 20.15%, nickel 28.10%, silicon 1.96%, manganese 0.64%, copper 3.02%, molybdenum 3.63%, columbium 0.79%, nitrogen 0.129%, and the balance of the alloy being substantially all iron. 20

12. A heat hardenable high corrosion resistance stainless steel alloy of the #20 type, said alloy having approximately the following chemical analysis: carbon 0.057%, chromium 20.15%, nickel 28.10%, silicon 1.96%, manganese 0.64%, copper 3.02%, molybdenum 3.63%, columbium 0.79%, nitrogen 0.129%, and the balance of the alloy being substantially all iron, the said alloy being adapted to be heat hardened to a BHN at least fifty points greater than that of a conventional #20 type alloy while retaining its high corrosion resistance. 25

13. A heat hardenable high corrosion resistance stainless steel alloy of the #20 type, said alloy having approximately the following chemical analysis: carbon 0.058%, chromium 19.75%, nickel 27.90%, silicon 1.92%, manganese 0.57%, copper 3.15%, molybdenum 3.95%, columbium 0.80%, nitrogen 0.250%, and the balance of the alloy being substantially all iron. 30

14. Two parts both made of high corrosion resistance stainless steel of the type known commercially as the #20 type (having an approximate analysis of 20% chromium, 28% nickel, 3.5% copper, and 3% molybdenum), said parts being used in combination, in sliding contact under pressure, one of said parts being the usual #20 alloy, solution annealed by heating and water quenching, and the other of said parts being made of an alloy of the #20 type having added thereto columbium and nitrogen, the columbium ranging from 0.20 to 1.00%, and the nitrogen ranging from 0.06 to 0.25%, hardened by heating, water quenching, and heat hardening, there being a difference in BHN hardness of at least fifty points, to prevent galling. 35

References Cited in the file of this patent

UNITED STATES PATENTS

- |           |                     |               |
|-----------|---------------------|---------------|
| 2,556,373 | Kirkby et al. ----- | June 12, 1951 |
| 2,587,613 | Payson -----        | Mar. 4, 1952  |